

## UNITED STATES PATENT OFFICE.

LOUIS FRIDERICH, OF GENEVA, SWITZERLAND, AND WILHELM RODENHAUSER, OF VOELKLINGEN-ON-SAAR, GERMANY, ASSIGNORS TO SIEMENS AND HALSKE, AKTIENGESELLSCHAFT, OF SIEMENSSTADT, GERMANY, A CORPORATION OF GERMANY.

## METHOD FOR THE DECARBONIZING OF HIGHLY-CARBONACEOUS FERROCHROMIUM.

No Drawing. Application filed September 5, 1925, Serial No. 54,793, and in Germany June 26, 1924.

The present invention relates to improvements in methods for the decarbonizing of highly carbonaceous ferro-chromium.

When producing ferro-chromium in electrical furnaces a product is obtained which usually contains 8-10 per cent carbon. Such ferro-chromium is however only available for few purposes on account of its high content of carbon. In many branches of the industry f. inst. in the high-grade steel industry for the producing of alloyed steel there is now a great demand for ferro-chromium which is as much as possible free from carbon, viz. a ferro-chromium having a carbon content below 1 per cent, or technically carbonless ferro-chromium with a carbon content of 0,5-0,2 per cent.

These high grade ferro-chromiums with a low content of carbon were hitherto produced in electric arc furnaces by melting highly carbonaceous ferro-chromium (which had been obtained in the usual way) together with chromium ores, whereby the ferro-chromium was refined. An exact control of this process is however not possible, wherefore the carbon content of the product obtained could not be fixed previously. It was therefore necessary in many cases to repeat the refining smeltings for several times in order to reduce the carbon content sufficiently. This is also the cause for the extraordinary costs of the ferro-chromium poor in carbon in comparison with the costs of the usual product.

According to the present invention the process is not carried out in an arc furnace but in an induction furnace, whereby the permanent reducing effect of the electric arc upon the charge—which hinders the refining—is avoided. At the new method it will neither be necessary to cool the highly carbonaceous ferro-chromium obtained at the first stage of operation before delivering it to the refining furnace and thereupon to smelt it anew. On the contrary the process according to the invention becomes especially advantageous and economical when carrying the same through with liquid ferro-chromium.

In its simplest form the invention consists in exposing the liquid charge to the influence of the oxygen of the air at a suitable temperature and without using any refining

or slag-forming agents. Hereby the surface of the bath must be kept clean (blank) so that the air may act unhindered upon the same.

The temperature during this process must be so high that an oxidation of the iron and the chromium is prevented. Preferably the temperature should be between 1425° C. and 1450° C. according to the contents of chromium. If the temperature becomes substantially higher than the above named limit the iron and the chromium will burn up and if the temperature becomes substantially lower no alloying will take place.

Scientific investigations have proved that at this method the decarbonizing takes place independently of the actual carbon contents of the charge and practically proportionally to the time used for the reaction. An essential saving of time is obtained in comparison to refining experiments performed with the best known slag coverings. At the present method it is also possible to analyze test quantities at any stage of the process in order to state the state of decarbonizing at any desired moment. A perpetual control of the process is thus possible. Experiments have further shown that the method may be carried out with a satisfactory result at any suitable lining in the furnace. Hitherto the best results have been obtained by a lining of chromite (chromic iron) and tar, because almost no wear occurs at this kind of lining. Another advantage lies in this, that the chromite simultaneously may be used as raw material for the producing of ferro-chrome.

This simple form of the method may be perfectionated in different ways.

An acceleration and perfection of the refining process may f. inst. be obtained through increasing the oxygen contents of the air layer over the bath surface by conducting artificial oxygen to the same. Hereby simultaneously the admission of nitrogen is prevented.

The nitrogen which is taken up in smaller or greater quantities at the process may also be removed by known means such as titanium, calcium, aluminium etc., a measure which also is applicable at other kinds of smelting furnaces.

The nitrogen may be excluded completely by adding oxygen delivering, easily decom-

posing, compounds such as super-oxides to the bath or by refining by means of steam, whereby oxygen is created through the dissociation which takes place on account of the 5 high temperature at hand.

What we claim as our invention and desire to secure by Letters Patent is:—

1. The process of producing low-carbon ferro-chromium by refining ferro-chromium 10 rich in carbon, which comprises heating the charge in an induction furnace, keeping the said charge at a temperature at which neither the iron nor the chromium will oxidize, exposing the clean surface of the bath to 15 the influence of the air over the same, and removing the nitrogen taken up during the process by adding to the charge a metal with great affinity to nitrogen.
2. The process of producing low-carbon 20 ferro-chromium by refining ferro-chromium rich in carbon, which comprises heating the charge in an induction furnace, keeping the said charge at a temperature at which neither the iron nor the chromium will oxidize, exposing the clean surface of the bath to 25 the influence of the air over the same, and adding oxygen delivering easily decomposing solid means such as super oxides to the charge.
3. The process of producing low-carbon 30 ferro-chromium by refining ferro-chromium rich in carbon, which comprises heating the charge in an induction furnace, keeping the said charge at a temperature at which neither the iron nor the chromium will oxidize, exposing the clean surface of the bath to 35 the influence of the air over the same, mixing an oxidizing gas to the said air, and removing the nitrogen taken up during 40 the process by adding to the charge a metal with great affinity to nitrogen.
4. The process of producing low-carbon ferro-chromium by refining ferro-chromium 45 rich in carbon, which comprises heating the charge in an induction furnace, keeping the said charge at a temperature at which neither the iron nor the chromium will oxidize, exposing the clean surface of the bath to 50 the influence of the air over the same, mixing an oxidizing gas to the said air, and adding oxygen delivering easily decomposing solid means such as super oxides to the charge.
5. The process of producing low-carbon 55 ferro-chromium by refining ferro-chromium rich in carbon, which comprises heating the charge in an induction furnace, keeping the charge at a temperature at which neither the iron nor the chromium will oxidize, exposing the clean surface of the bath to 60 the influence of the air above the same and leading steam into the said air.
6. The process of producing low-carbon ferro-chromium by refining ferro-chromium 65 rich in carbon, which comprises heating the charge in an electric induction furnace, keeping the said charge at a temperature at which neither the iron nor the chromium will oxidize, exposing the clean surface of the bath to the influence of the air above the same, leading steam into the said air, and removing the nitrogen taken up during the process by adding to the charge a metal with great affinity to nitrogen.
7. The process of producing low-carbon 70 ferro-chromium by refining ferro-chromium rich in carbon, which consists in heating a lining of chromite in an electric induction furnace, keeping the charge at a temperature at which neither the iron nor the chromium will oxidize, exposing the clean surface of the bath to the influence of the air above the same, and removing the nitrogen taken up during the process by adding to the charge a metal with great affinity to nitrogen.
8. The process of producing low-carbon 75 ferro-chromium by refining ferro-chromium rich in carbon, which comprises heating a lining of chromite in an electric induction furnace, keeping the charge at a temperature at which neither the iron nor the chromium will oxidize, exposing the clean surface of the bath to the influence of the air above the same, and removing the nitrogen taken up during the process by adding to the charge a metal with great affinity to 80 nitrogen.
9. The process of producing low-carbon 85 ferro-chromium by refining ferro-chromium rich in carbon, which comprises heating a lining of chromite in an electric induction furnace, keeping the charge at a temperature at which neither the iron nor the chromium will oxidize, exposing the clean surface of the bath to the influence of the air above the same, and adding oxygen delivering easily 90 decomposing solid means such as super oxides to the charge.
10. The process of producing low-carbon 95 ferro-chromium by refining ferro-chromium rich in carbon, which comprises heating a lining of chromite in an electric induction furnace, keeping the charge at a temperature at which neither the iron nor the chromium will oxidize, exposing the clean surface of the bath to the influence of the air above the same, leading steam into the said air, and adding to the charge a metal with great affinity to 100 nitrogen.
11. The process of producing low-carbon 105 ferro-chromium by refining ferro-chromium rich in carbon, which comprises heating a lining of chromite in an electric induction furnace, keeping the charge at a temperature at which neither the iron nor the chromium will oxidize, exposing the clean surface of the bath to the influence of the air above the same, leading steam into the said air, and removing the nitrogen absorbed during the process by adding oxygen delivering easily 110 decomposing solid substances such as super oxides to the charge.
12. The process of producing low-carbon 115 ferro-chromium by refining ferro-chromium rich in carbon, which comprises heating a lining of chromite in an electric induction furnace, to a temperature in the neighborhood of 1425-1450° C., keeping a clean surface of the bath and exposing the said clean surface to the influence of an oxidizing gaseous medium.

12. The process of producing low-carbon ferro-chromium by refining ferro-chromium rich in carbon, which comprises heating a lining of chromite in an electric induction furnace, keeping the charge at a temperature in the neighborhood of 1425-1450° C., exposing the clean surface of the bath to the influence of the air over the same, and removing the nitrogen taken up during the process by adding to the charge a metal with great affinity to nitrogen. 35
13. The process of producing low-carbon ferro-chromium by refining ferro-chromium rich in carbon, which comprises heating a lining of chromite in an electric induction furnace, keeping the charge at a temperature in the neighborhood of 1425-1450° C., exposing the clean surface of the bath to the influence of the air over the same, and adding 40 oxygen delivering easily decomposing means such as super oxides to the charge. 50
14. The process of producing low-carbon ferro-chromium by refining ferro-chromium rich in carbon, which comprises heating a lining of chromite in an induction furnace, keeping the charge at a temperature in the neighborhood of 1425-1450° C., exposing the clean surface of the bath to the influence of the air above the same and leading steam into 55 the said air. 60
15. The process of producing low-carbon ferro-chromium by refining ferro-chromium rich in carbon, which comprises heating in
- an electric induction furnace a lining of chromite and a binding agent, keeping the charge at a temperature in the neighborhood of 1425-1450° C., exposing the clean surface of the bath to the influence of the air above the same, and removing the nitrogen taken up during the process by adding to the charge a metal with great affinity to nitrogen. 40
16. The process of producing low-carbon ferro-chromium by refining ferro-chromium rich in carbon, which comprises heating a lining of chromite in an electric induction furnace, a lining of chromite and a binding agent, keeping the charge at a temperature in the neighborhood of 1425-1450° C., exposing the clean surface of the bath to the influence of the air above the same, and adding oxygen delivering easily decomposing solid substances such as super oxides to the charge. 50
17. The process of producing low-carbon ferro-chromium by refining ferro-chromium rich in carbon, which comprises heating a lining of chromite and a binding agent in an electric induction furnace, keeping the charge at a temperature in the neighborhood of 1425-1450° C., exposing the clean surface of the bath to the influence of the air above the same, and leading steam into the said air. 60

In testimony whereof we affix our signatures.

LOUIS FRIDERICH.  
WILHELM RODENHAUSER.